

Patented Aug. 9, 1927.

1,638,273

# UNITED STATES PATENT OFFICE.

ALADAR PACZ, OF EAST CLEVELAND, OHIO.

## METHOD AND COMPOSITION OF MATTER FOR SURFACE-TREATING ALUMINUM.

No Drawing.

Application filed February 10, 1926. Serial No. 87,463.

This invention relates to the surface treatment of aluminum articles for the purpose of ornamenting the same or of rendering the same more resistant to corrosion and is applicable either to articles of pure aluminum or to alloys in which aluminum is a preponderent ingredient. The process involves as its main feature the subjection of such aluminum surface or article to the simultaneous action of a soluble fluo-silicate, a salt of a non-ferrous, iron-group, metal, and an alkali salt. The fluo-silicate employed is preferably that of sodium which is the cheapest and most readily available, although I do not limit myself thereto; a very convenient, satisfactory and effective concentration in practical use is that wherein the bath contains 0.15% of this material, but I do not limit myself to this strength. By non-ferrous, iron-group, metal I intend to designate nickel and cobalt and any convenient salt thereof can apparently be used. I have had excellent success with the sulphate, nitrate, and chloride of these metals. A very convenient and practical concentration of the same is from 0.2% to 0.3%, although I do not limit myself thereto. By alkali salt I designate salts both of the fixed alkalies and of the volatile alkali, and the particular salt which I prefer to use is the nitrate although I have had a measurable degree of success with such other salts as the phosphate and sulphate. In using ammonium, sodium, or potassium nitrate I have found that 1% is a very satisfactory concentration although I do not limit myself thereto. It appears to be necessary that this third ingredient be preponderant.

The solution is preferably employed hot, even up to the boiling point, and the articles to be treated are immersed therein for a greater or less length of time as determined by the extent of treatment desired which can readily be judged by the eye. The effect of this treatment is to produce upon the surface a mottled, speckled, or spotted appearance, irregular portions of varying sizes and shapes being covered with a dense adherent, dark, deposit intermingled with streaks and ridges of bright and unaffected aluminum color. In general the more concentrated the solution or the higher the temperature the smaller are the spots and the finer grained the design; and also the more rapidly the process is performed. Variations in the relative quantities of the ingredients

also affect the size of the grain and the manner of the ornamentation. Thus an increase in the amount of the fluo-silicate produces a finer grain and a decrease tends to coarsen the same. An increase in the amount of the iron group metal produces a much similar change of the graining. The effect of the alkali salt appears more especially to influence the strength or depth of the colorization which becomes faint with low concentrations and darker and blacker with greater strengths.

The resulting coating is unaffected by heat and is highly resistant to abrasion even that of a steel brush, the unmodified aluminum surface yielding rather than the modified or coated portion. By the use of proper concentrations and temperatures the surface can be very thoroughly covered with the coating described. Care however, must be observed not to permit too great proximity between metallic articles receiving simultaneous treatment. Stencils or other protective means can be employed if desired to shield any desired portion against the action of the solution. The solution can be used repeatedly although additions of the several ingredients are required from time to time. Eventually the solution becomes sufficiently contaminated with impurities, partly dissolved from the articles and partly of accidental entrance so that it must be discarded.

The articles after receiving the treatment hereinbefore described can be subjected, if desired, to further treatments designed to color the unmodified portions, or may be covered with paint, lacquer, etc., which adheres much more strongly thereto than to the unmodified metal.

Alloys of aluminum with other metals, such as silicon, magnesium, zinc, copper and the like are likewise susceptible to this process, although in many cases the surface does not exhibit the striking contrast between the color of the modified and unmodified portions which is presented by pure aluminum. For example an alloy of aluminum and silicon treated in this manner exhibits areas of lead color interspersed with areas of a comparatively light grey, the whole resembling marble.

It will be understood that I do not limit myself to the concentrations herein described nor to the particular salts above enumerated except within the limits specifically indi-

cated. It is necessary to the successful performance of my process to employ the combined effect of the three types of ingredients, but each of said ingredients can be varied within its own class and I do not limit myself except as specifically set forth in my several claims.

Having thus described my invention what I claim is:

10 1. The process of surface treating metallic articles consisting at least superficially of aluminum which contains the step of immersing the article in a solution containing a soluble fluo-silicate, a salt of a non-ferrous 15 iron-group metal; and an alkali salt.

20 2. The process of producing an irregularly mottled aluminum surface which contains the step of subjecting a clean aluminum surface to the simultaneous action of a soluble fluo-silicate, a salt of a non-ferrous iron 25 group metal, and an alkali nitrate.

3. The process of providing aluminum articles with a hard, permanent surface which contains the step of subjecting the same to the action of a relatively dilute solution containing three types of ingredients, one of which is a soluble fluo-silicate, the second a metallic salt, and the third a neutral alkali salt.

4. As a composition of matter, a dipping solution for aluminum articles containing a soluble fluo-silicate, a soluble metallic salt, and a neutral alkali salt.

5. As a composition of matter, a dipping solution for aluminum articles comprising a soluble fluo-silicate, a soluble salt of a non-ferrous metal of the iron group, and an alkali nitrate, all dissolved in water.

In testimony whereof I hereunto affix my signature.

ALADAR PACZ.